

July 3, 1934.

H. BARNETT

1,964,806

BOTTOM FILLER

Filed Oct. 29, 1930



INVENTOR  
Herbert Barnett  
By his Attorney,  
Harlow M. Davis

## UNITED STATES PATENT OFFICE

1,964,806

## BOTTOM FILLER

Herbert Barnett, Leicester, England, assignor to  
 United Shoe Machinery Corporation, Paterson,  
 N. J., a corporation of New Jersey

Application October 29, 1930, Serial No. 491,983  
 In Great Britain November 27, 1929

4 Claims. (Cl. 106—3)

This invention relates to improvements in shoes and to bottom fillers therefor and is disclosed herein with reference to a cold filler adapted to be applied when in plastic condition to the insole of a shoe and to be spread upon the insole before the outsole is attached.

In the manufacture of shoes it is usual to fill the space between an inner and an outer sole and within the margin of the shoe upper by means of a filler which may be a shaped piece of felt, leather-board or the like, but which at the present time is often, and usually in the case of welt shoes, a compound of a solid material (such as cork or the like, granulated, comminuted or otherwise finely divided) with an adhesive or binder which is, or may be made, more or less fluid so that the compound may be applied while plastic. These compounds as usually used may be divided into two broad classes, namely, hot method fillers and cold method fillers. In the case of the hot method filler the compound is normally in a practically solid condition and is heated when it is desired to make it plastic for application to the shoe after which application it is allowed to set again. In the case of the cold method filler the compound, in addition to cork or other solid material, usually comprises an adhesive or binder in the nature of a rubber solution (i. e. a solution of solid rubber in a volatile solvent, for example naphtha) so that the compound is normally plastic and becomes set by the evaporation of the solvent from the binder. The usual hot method filler involves the use of heating apparatus and considerable time if char-ring of the solid material (e. g. cork) is to be prevented and also is liable under the pressure and the heat of the foot during wear to alter its form or position to an uncomfortable degree (the binder being of the nature of glue), while the usual cold method filler by reason of the nature of the solvent used involves the danger of fire and consequently requires precautions which many shoe manufacturers are unwilling to take. On the other hand a filler comprising such a rubber or rubber-like binder as referred to has the advantage that no auxiliary apparatus is necessary to bring it to a workable condition.

Theoretically an ideal compound shoe bottom filler should have the following qualities:—it should not require any special precautions in factory storage or use; it should not deteriorate under conditions liable to be met with in ordinary shoe factories; it should be pliable or plastic at ordinary temperatures; it should be easily workable; it should set quickly when put in place

on the shoe bottom in order not to delay factory operations; it should, when set, not be brittle or friable nor likely permanently to alter its form or position to any great extent under the pressure and heat of the foot; it should be sufficiently flexible when set to accommodate itself readily without deterioration to the flexure of the shoe in walking; it should be resilient; it should be substantially waterproof; it should be unaffected by change of climate; it should be odorless; it should be sufficiently adhesive to adhere adequately to the shoe parts when placed in position; it should be economical in first cost and in cost of application; and it should be such as not to act detrimentally upon the shoe parts. Heretofore, a large number of fillers have been suggested each of which has certain advantages but is lacking to some degree at least in other desirable qualities.

It is an object of the invention to provide an improved shoe bottom filler having so far as is possible the qualities of the theoretical ideal referred to above.

In one of its aspects the invention provides a compound shoe bottom filler which comprises a binder of rubber latex adhesive, that is, an adhesive that includes a substantial amount of rubber in the form of latex, together with suitable comminuted solid material, for example cork. Rubber latex adhesives have various forms, being sometimes merely a natural latex of one or more closely allied varieties of rubber (such as hevea) with the mere addition of a coagulation preventative. Such an adhesive is represented by many of those known commercially as "rubber latex". In other cases other materials are added in greater or lesser proportions, for example with the object of modifying the normal setting or the adhesive qualities of the adhesive.

In order to increase the adhesive qualities of the latex bottom filler so that it will stick more firmly to the shoe bottom when it is first applied and before it has had time to set or solidify, a suitable resin, for example in the form of a soap made by treating rosin with concentrated ammonia, may be added to the latex before the latex is mixed with the cork. The addition of a volatile rubber solvent to the latex and cork filler is also advantageous since it reduces the amount of latex required for a given amount of cork and results in a filler which is more flexible after it has become set.

As hereinafter used the term "latex" is intended to cover not only natural latices, with or

without modification as described above, but also artificial water dispersed rubber cements, as distinguished from the well-known type of cement in which the rubber is dissolved in a readily 5 volatile organic solvent such as naphtha.

In another aspect the invention comprises a shoe having between its insole and its outsole a bottom filler comprising comminuted solid material rendered plastic by the addition of latex, 10 with or without other materials.

With the above and other objects in view the invention will now be described in connection with the accompanying drawing and pointed out in the claims.

15 The drawing illustrates a shoe the bottom of which is provided with a filler in accordance with the present invention.

While the proportions of the ingredients used in making a bottom filler in accordance with my 20 invention may be varied considerably the following describes the compounding of a typical sample of such filler. Commercial rubber latex having a rubber content of perhaps 40% is added to ground cork and the two are thoroughly mixed 25 so that the latex is diffused throughout the cork, enough of the latex being used to form a doughy mass. The proportions of the ingredients necessary will, of course, vary with variations in the 30 composition of the latex and the fineness of the cork.

If it is desired to form a filler which will be more tacky and will, therefore, stick better to the shoe bottom when freshly applied and before it has had time to set, then a resin soap is made, 35 for example by adding one part of rosin to two parts of concentrated ammonia (specific gravity .880), and is added to the latex before the latter is mixed with the cork.

If a more flexible filler than that just described is desired a volatile rubber solvent may be added after the latex and cork have been mixed. In order to eliminate fire hazard this solvent should be of a non-inflammable nature such as carbon tetrachloride, cyclohexone, etc. 45 For example, 8 gallons of carbon tetrachloride may be added to a dough consisting of 18 pounds of ground cork into which has been worked 14 pounds of latex. To produce a cheaper product naphtha or benzol may be used in place of the carbon tetrachloride mentioned in the foregoing example, though that, of course, increases the fire risk.

The filler manufactured as above may be packed into cans and kept in that manner until it is to be used.

The accompanying drawing illustrates a Good-year welt shoe having an upper 2, an insole 4, a

welt 6 and an outsole 8, the space at the forepart of the shoe between the insole 4 and the outsole 8 being filled, as illustrated at 10, with a filler compounded in accordance with my invention and comprising particles of ground cork 12 which are caused to adhere to each other by the rubber of the latex, and the resin, if such has been added, which fills the interstices between the cork particles 12, as indicated at 14. In making such a shoe the filler is spread cold on the insole of the shoe after the sole and welt have been stitched to the lasted upper and insole and when the shoe is otherwise ready for the attachment of the outsole.

If desired other suitable comminuted solid material, for example wood fibre or leather fibre, may be used in place of some or all of the ground cork described above. Other resin soaps than that described above may be also used. The soap may be formed by adding rosin to other alkalis than ammonium, for example to a soda solution. Other resins such as copal and dammar also may be used for this purpose, though rosin is entirely satisfactory and much cheaper.

90 If desired the materials described above may 100 be formed into sheets and dried or allowed to dry, suitably shaped pieces being subsequently die cut from the sheet material to be used as sheet bottom filler in the manufacture of shoes.

Having thus described the invention, what I 105 claim as new and desire to secure by Letters Patent of the United States is:

1. A shoe bottom filler comprising a comminuted solid, a binder of latex and a resin soap in proportions to provide a tacky substance of 110 a degree of plasticity which permits it to be spread readily by hand throughout the cavity in a shoe bottom.

2. A shoe bottom filler comprising a comminuted solid, a binder of latex, a resin soap and a 115 volatile rubber solvent in proportions to provide a tacky substance of a degree of plasticity which permits it to be spread readily by hand throughout the cavity in a shoe bottom.

3. A shoe bottom filler comprising a comminuted solid, a binder of latex, a resin soap and carbon tetrachloride in proportions to provide a 120 tacky substance of a degree of plasticity which permits it to be spread readily by hand throughout the cavity in a shoe bottom.

4. A shoe bottom filler comprising a comminuted solid, a binder of latex, a resin soap and benzol in proportions to provide a tacky substance of a degree of plasticity which permits it to be spread readily by hand throughout the 130 cavity in a shoe bottom.

HERBERT BARNETT.